

## UNITED STATES PATENT OFFICE

2,415,036

## RESISTANCE MATERIAL

Archibald C. Quinn, Detroit, Mich., assignor to  
 Bendix Aviation Corporation, Detroit, Mich., a  
 corporation of Delaware

No Drawing. Application October 13, 1944,  
 Serial No. 558,611

5 Claims. (Cl. 201—76)

1

This invention relates to electrical resistance material.

Broadly the invention comprehends a new material for the production of resistance units such as are used in electrical circuits.

An object of the invention is to provide an electrical resistance of such material that the voltage or flow of current may be satisfactorily regulated.

Another object of the invention is to provide a satisfactory material for the manufacture of resistance units such as are used in making-and-break switches, the material being characterized in that the possibility of arcing of the switch is inhibited.

Another object of the invention is to provide a highly efficient electrical resistance element made of metal and glass powders intimately mixed.

It has been found that an electrical resistance element proves eminently satisfactory for general use in electric circuits when the element is made of a material derived from a compound of metal and glass powders. In the preparation of the resistance material through the use of metal and glass powders, a critical percentage of metal is essential before the material becomes conductive. In instances where either copper or nickel powder is used of a —325 mesh, a minimum of forty-two per cent (42%) of metal is found to be essential.

In practice, the maximum specific resistance thus far attained in the usage of copper and glass, and nickel and glass is—

Ohm. cm.

Copper and glass..... 025  
 Nickel and glass..... 125

Although these values have been obtained, they are by no means static. The percentage of metal used and the resultant specific resistance is controlled by the mesh size of both constituents, the thoroughness of mixing the constituents, and the manner of curing the material, that is, the heat treatment of the compound.

The specific resistance of a copper and glass mixture and a nickel and glass mixture, both containing the same percentage of metal, are quite different. This is due to the specific resistance of the raw metals; as, for example—

Ohm. cm.

Copper..... —.0000017  
 and  
 Nickel..... —.0000078

2

However, it is to be clearly understood that the invention is not limited to the use of copper and nickel. As to the metallic element of the material, any other metal may be employed with excellent results.

Although the resistance obtained through the use of a mixture of copper and glass, and also a mixture of nickel and glass, is much higher than in instances where pure nickel or copper elements are used, in some instances it is necessary to obtain higher resistances than obtainable with either of the above compositions.

It has been discovered that with the addition of silicon as a third element in the compound, the resistance values are enormously increased. This is clearly shown by actual tests; as, for example, a compound of—

|         | Per cent |
|---------|----------|
| Copper  | 40       |
| Silicon | 10       |
| Glass   | 50       |

has a resistance value of 1.17 ohm. cm.; and a compound of

|         | Percent |
|---------|---------|
| Nickel  | 35      |
| Silicon | 15      |
| Glass   | 50      |

has a resistance of 3.10 ohm. cm. A material composed of silicon 25% and glass 75% has a resistance value of 1,000,000 ohm. cm. Thus, the value of silicon has a constituent of the compound becomes clearly evident.

Through the use of a compound of glass, silicon and metal, preferably copper or nickel, a resistance material may be varied through wide limits. The variation of resistance may be obtained in the following manner; i. e., by keeping the percentage of glass constant and varying the percentage of silicon and nickel; by keeping the silicon constant and varying the percentage of nickel and glass; by keeping the nickel constant and varying the percentage of silicon and glass; and also by varying the particular mesh of the respective constituents of the compound.

It has been found that a highly satisfactory resistance bar may be had by compounding the following materials in the percentages given; i. e.—

|                | Parts |
|----------------|-------|
| Powdered glass | 57.5  |
| Silicon metal  | 8.0   |
| Nickel metal   | 34.5  |
| Paraffin wax   | 7.5   |

55 In preparing this compound the wax is dissolved

in carbon tetrachloride. The metal powders and glass powder are then mixed and added to the wax solution. This mixture is placed in a ball mill and more carbon tetrachloride is added to form a thin slurry. The mixture is then thoroughly milled, drained off, and dried. When thoroughly dried, it is screened through a fine mesh screen. The material is loaded into a steel die and compressed to the contour of the piece desired. In order to remove volatile constituents from the pressed bar, it is then sintered at a low temperature; for example, 1000° F. for fifteen minutes. Then, to attain the desired physical characteristics of the bar, it is re-sintered at a higher temperature; for example, 1600° F. for fifteen to thirty minutes.

While this invention has been described in connection with certain specific embodiments, the principle involved is susceptible of numerous other applications that will readily occur to persons skilled in the art. The invention is, therefore, to be limited only as indicated by the scope of the appended claims.

Having thus described the various features of

the invention, what I claim as new and desire to secure by Letters Patent is:

1. A resistance material comprising powdered glass 50%, powdered copper 40%, and powdered silicon 10%.
2. A resistance material comprising a compound of glass powder 50%, nickel powder 35%, and silicon powder 15%.
3. A resistance material comprising the following constituents compounded in the proportions given: powdered glass 57.5 parts; powdered silicon 8.0 parts, and powdered nickel 34.5 parts.
4. A resistance bar comprising a compound of powdered glass 57.5 parts, powdered silicon 8.0 parts, powdered nickel 34.5 parts, and paraffin wax 7.5 parts, in solution, thoroughly mixed, dried, compacted, and sintered.
5. The method of producing a resistance bar comprising compounding glass powder 57.5 parts, silicon powder 8.0 parts, nickel powder 34.5 parts, and paraffin wax 7.5 parts, drying the mixture, compacting the mixture to form the bar, and sintering the bar.

ARCHIBALD C. QUINN.